

## UNITED STATES PATENT OFFICE

1,939,390

STEEL ALLOY AND PROCESS OF MAKING  
SAME

John L. Cox, Philadelphia, Pa.

No Drawing. Application October 27, 1928  
Serial No. 315,593

18 Claims. (Cl. 75—1)

My invention relates to a steel alloy for use at high temperatures which is especially suited for the manufacture of valves for internal combustion engines. Valves of this character in use are subject to conditions which tend rapidly to reduce their efficiency and shorten their life. The high temperature to which they are subjected has the effect of softening and of scaling the valve heads, so that they deform readily and do not seat properly. Under the influence of heat, the valve stems tend to seize in their bearings. Some steels which are otherwise fairly satisfactory at high temperature are too soft to withstand the blows of the tappets upon the ends 15 of valve stems made from them, which therefore tend to upset and fail to function properly.

Another cause of failure in such valves is the alteration of size which occurs in passing from the alpha to the gamma state and vice versa. 20 Most valve steels possess a critical temperature so low that a valve on going into service is heated above its critical range, becoming austenitic in structure. Cooling quickly after use, the valve becomes martensitic, increasing in size. Reheated to the gamma range on resuming work, the valve shrinks again. This alternation of size has a tendency to crack the valves.

A valve having the composition herein disclosed is substantially free from these causes of 25 deterioration and can be manufactured at a moderate cost.

A valve embodying my invention is composed of steel alloyed with nickel, chromium and aluminum, in suitable proportions hereinafter specified, to which are added silicon and manganese in proportions not necessarily substantially different from those characterizing known steel alloys.

I have found that aluminum, added to a nickel-chromium steel, has for one effect that of raising its critical temperature in the proportion, roughly, of 70° F. for each one per cent. of aluminum, which is contrary to the belief held by high authority that aluminum must reduce the critical 40 temperature of steel. Further, aluminum, through its production on oxidation of a thin film of adherent oxide, serves to protect from oxidation the other elements with which it is alloyed.

Nickel in such a combination has for one effect the lowering of the critical temperature of transformation of carbon steel at a rate of about 14.5° F. for each per cent. of nickel. In steels with about 10 per cent. of chromium, the effect is 45 much more marked and the transformation tem-

perature is lowered about 50° F. for each addition of 1% of nickel. Its advantages lie in the increased hardness of the alloy, increased resistance to oxidation, in its production of a tightly adherent scale, and in the fact that in a 60 chrome-aluminum valve it prevents seizing and galling of the valve stem in its guides.

Furthermore, nickel and aluminum possess the property of combining to form an exceedingly hard alloy having the composition NiAl, which 65 retains its hardness at elevated temperatures.

Chromium in high percentages in steel has the effect of increasing the strength of the steel at high temperatures and of strongly resisting oxidation.

While certain of the specified characteristics and actions of the metals designated are known, it is believed that other characteristics and actions, especially the effects of associating one metal with another and of adjusting the proportions of the various metals, have not heretofore been known. Certainly their practical application to the solution of the difficult problem of manufacturing valve steel has never occurred to those skilled in the art. With the knowledge, in 70 part known and in part discovered by me, of these absolute and relative qualities, I have found it possible, by a judicious combination of the amounts of nickel, chromium and aluminum, to produce steels that will meet all the exacting requirements for valves. Thus, I have found it 75 possible, by suitably varying proportions, to give to the steel critical temperatures of transformation higher than the operating temperatures to which different valves are subjected. Further, 80 up to a proportion of aluminum which will render the alloy brittle, say about 7%, the hardness can be increased by increasing the nickel content 85 correspondingly, but always at the expense of lowering the critical temperature, which may be 90 necessary to permit hardening the ends of the stems.

The proportions of nickel may vary within a wide range, say from .5 or .75 to 8%, but is preferably less than 4%. The proportion of chromium 100 may also vary widely, say from 6% to 15%, but is preferably less than 10%. The proportion of aluminum may vary from .5 to 7%, although the most desirable percentage is from 1.5 to 3.5%. The proportion of silicon may vary from .3 to 105 4%, although a range of 1% to 1.8% is preferred. The proportion of manganese may vary from .25 to 2%, although .35 to .65% is preferred. These proportions of silicon and manganese do not 110

substantially differ from those within the known or usual range of alloy steel making practice.

The most desirable percentage of carbon is from .3 to .6%, although this percentage may be reduced to .25% and, in special cases, raised to 1.25%. Ordinarily, however, the carbon content should not exceed .75%.

It must be borne in mind, however, that the proportions of certain of the ingredients should not be varied arbitrarily within the ranges specified, but certain of them should have certain ratios, variable within limits, and dependent on the qualities, especially the critical temperature, desired.

I submit herewith, in the first three columns, three specific valve compositions, in the fourth column a desirable range of proportions, and in the last column what may be considered, except perhaps in very special cases, an extreme range of proportions:

|     |      |      |     |            |             |
|-----|------|------|-----|------------|-------------|
|     | .57  | .48  | .4  | .35 to .60 | .25 to 1.25 |
| Cr. | 8.60 | 9.30 | 9.5 | 8 to 12    | 6 to 15     |
| Ni. | 3.33 | 1.18 | 1.2 | 1 to 3.5   | .5 to 8     |
| Al. | 3.28 | 2.12 | 1.8 | 1.5 to 2.5 | .5 to 5     |
| Mn  | .42  | .61  | .4  | .35 to .65 | .2 to 2     |
| Si. | .40  | 1.05 | 1.5 | 1 to 1.8   | .3 to 4     |

Compositions not varying widely from the second composition are, perhaps, preferable for most uses.

In these compositions, as previously stated, the aluminum has a distinct hardening effect through the nickel which is present and which is entirely different from its action upon alloys free from nickel, and it raises the critical hardening range, which tends to keep the valve head from cracking due to change of size in passing through this range.

Furthermore, the material is exceptionally resistant to scaling at high temperature, and the scale which forms has a tendency to adhere to the metal and not drop off. This is of great advantage in securing continuous good seating of a valve.

By heating to a very high heat and then quenching the end, the valve stem, moreover, is sufficiently hard to withstand the blows of the tappets.

Notwithstanding all the above advantages, the composition does not contain expensive ingredients in high proportions, permitting the manufacture of valves at reasonable cost.

It is believed that the composition herein disclosed is novel, but it should be understood that aside from the novelty of the composition, specific novelty also resides in the discovery that said composition is especially adapted to the manufacture of valves, in that valves of the disclosed composition possess a combination of qualities and advantages that have never hitherto characterized any alloy steel that is marketable at a reasonable price, and that the especial adaptability of the disclosed composition to the manufacture of valves, as distinguished from numerous other articles that are fabricated from alloy steels of various composition, is not obvious and cannot be determined without thorough tests under adverse conditions.

In determining the proportions of certain ingredients, the temperature conditions to which the valves are subjected should be borne in mind. Some valves, as, for example, those used in Diesel engines, are subjected to a much lower maximum temperature than the valves used in airplane engines. The required critical temperature of

the steel may vary from 1400° to 1800° or possibly 1900° F. Starting with a chromium alloy steel having a critical temperature of about 1600° F., my experiments, for which a certain margin of error must be allowed, indicate that not only must sufficient nickel and aluminum be added to secure the known functions of nickel and aluminum respectively, but they must be added in proportions more or less nearly equal to maintain that critical temperature. The permissible proportion of each may vary widely provided substantial equality of proportions is maintained between them. If the critical temperature of the alloy is permissibly substantially less than 1600° F., the ratio of aluminum to nickel should be substantially reduced, while if a higher critical temperature is required the ratio of aluminum to nickel should be substantially increased. The following table discloses the approximate nickel-aluminum relationship as applied to a chromium steel alloy having a critical temperature of about 1600° F.:

With a ratio of about 1:1 (Ni to Al) critical temperature remains at 1600° F.  
With a ratio of 1:0.4 (Ni to Al) critical temperature becomes 1500° F.  
With a ratio of 1:0.9 (Ni to Al) critical temperature becomes 1700° F.  
With a ratio of 1:2.75 (Ni to Al) critical temperature becomes 1800° F.  
With a ratio of 1:3.90 (Ni to Al) critical temperature becomes 1900° F.

It should be understood that this table is based on my own experiments and that other experiments may yield a somewhat different result; but the table is reliable as indicating, with an approximation to accuracy, the effects of varying the ratios of nickel to aluminum.

It should also be understood that, as before explained, the presence of chromium, which as before explained affects materially the critical temperature reducing effect of nickel, affects the required ratios between nickel and aluminum, and that therefore the greater the percentage of chromium, the smaller the permissible percentage of nickel, in order to secure a given critical temperature for the alloy. The presence of chromium thus affects the required ratio between nickel and aluminum.

It should also be understood that the percentage of silicon affects the critical temperature, that my composition requires no high silicon content, and that it is possible to produce alloy steel embodying my invention and containing a percentage of silicon that is within the lower part of the range of alloy steel making practice. Since silicon and manganese are present in nearly all carbon steels, my invention may be said to comprise, broadly, the addition, to carbon steel (of which the carbon content should generally be less than one per cent.), of chromium 6 to less than 15%, nickel .5 to 8% and aluminum .5 to 7%; the proportions of aluminum and nickel, and also the ratio of one to another, varying with the critical temperature desired, as above explained. While the percentage of carbon may, in exceptional cases, exceed one per cent., valves that will meet requirements to the fullest degree should comprise the constituents named in the following proportions: carbon not over about .75% or under about 0.25% and preferably from 0.35 to .6%; nickel, between 1 and 4%, preferably not over 3.5%; chromium within, or at any rate not far outside, the range 8 to 11 or 12%; and aluminum 1 to 4% and preferably with the range 1.5% to 2.5%.

While the proportions of the different ingredients may vary within a fairly wide range, it

must be understood, as hereinbefore explained, that a low or high percentage of one ingredient may not be associatable with respectively high or low percentages of every other ingredient. 5 This is particularly true of aluminum in its relation to nickel, and to nickel and chromium combined. Thus, the percentage of nickel should not be in excess of 2.5 times the percentage of aluminum; and in most instances the percentage of aluminum should not be substantially less, or should substantially exceed, the percentage of nickel, as in the specific illustrative compositions hereinbefore given. So, also, the percentage of aluminum should be at least one-ninth, and usually should be at least one-sixth, the percentage of nickel and chromium combined.

There is no novelty in the present process so far as concerns the procedure of mixing the ingredients, melting, heat treating, etc., which may follow established practice of making steel alloys, the novelty residing in the proportioning of the ingredients and in varying such absolute and relative proportions in accordance with the critical temperature desired.

25 I am aware of the fact that alloys are known containing chromium from 15 to 25%, nickel from 5 to 10%, aluminum from  $\frac{1}{2}$  to 2%, and high carbon above 1%, the ratio of aluminum to nickel varying from 1 to from 5 to 10. Such alloys are intended for heavy castings, such as parts of oil stills, and it is not practicable to forge them, nor are they intended to be forged. They are said to be of value where rigidity under a heavy load at high temperatures is a desideratum. 35 They are, however, wholly valueless to secure the qualities desirable in valves and in other forged articles subject to similar requirements and conditions of use. I am also aware of the fact that alloys are known containing chromium 10 to 15%, nickel 4 to 10%, and titanium .2 to 4%, with ordinary proportions of silicon and manganese. The only aluminum that is said to be permissive in such alloys is that very small proportion which is present in the ferro-chrome if it is made by the thermite process. Such alloys are said to be malleable only if the carbon be reduced as low as .11 or .12% and easily machinable only if the carbon is reduced to about .08%. In my composition, the percentage of nickel rarely approximates as high as four per cent.; the amount of aluminum is rarely less than 40% of the amount of nickel and when a medium or high critical temperature is desired the percentage of aluminum substantially exceeds the percentage of nickel; and although the percentage of carbon is never less than .2% and is usually between .35 and .60% and may approximate .1%, the alloy is both malleable and machinable.

60 I also disclaim as my invention any composition containing 5% or more of nickel, unless the percentage of nickel is less than 2.5 times the percentage of aluminum. Exceptionally, an alloy containing as high as 5%, but not over 8%, nickel will have, in degree, qualities characteristic of my invention; but in no case will it possess such qualities if the proportion of nickel to aluminum exceeds that specified. A composition defined, broadly, as containing, as essential alloying ingredients, chromium and aluminum in any defined proportions and 5% or more of nickel, without the above limitation to relative percentages of nickel and aluminum, is disclaimed as my invention.

75 My composition, therefore, depends for its

novelty on proportions of the constituent metals, and although these are variable within fairly wide ranges, they cannot be varied to the extent that all the ingredients of the composition would be brought within the ranges above specified. 80

The requirements of a perfect valve, namely, resistance to scaling at high temperature, resistance to upsetting and deformation, prevention of seizure in their bearings, and maintenance of structure and size and shape under high temperatures with subsequent cooling, are all possessed by valves constructed in accordance with my composition, although the required combination of qualities is entirely absent if the desirable proportions of the ingredients are departed from to a degree that would produce an alloy whose ingredients are within the proportions of known alloys composed of the same metals. Thus, in the known alloy to which reference is made, while great hot hardness is secured by the high nickel and high carbon content, the association of these ingredients with a high chromium content and an aluminum content that is low compared with the nickel content would reduce the critical temperature of the alloy below a practicable limit, making the steel austenitic at ordinary temperatures, and would fail to approximate the other desired valve characteristics even as closely as other valve compositions heretofore known.

90 What I claim and desire to protect by Letters Patent is:

1. A hard steel alloy containing carbon about .2 to less than 1%, nickel about .5 to 8%, chromium about 6 to less than 15%, and aluminum about .5 to 7%, the remainder being substantially iron, the percentage of nickel being less than 2.5 times the percentage of aluminum; said alloy having a critical temperature not less than about 1400° F. and having the characteristics of resistance to alterations in structure, size and shape with great temperature changes, retention of hardness at elevated temperatures, freedom from scaling, resistance to deformation, and which is readily malleable and machinable. 100

110 2. A hardened valve adapted for use in internal combustion engines and composed of a readily malleable and machinable steel alloy having a critical temperature not less than 1400° F. and containing carbon about .2 to less than 1%, nickel about .5 to 8%, chromium about 6 to less than 15%, and aluminum about .5 to 7%, the remainder being substantially iron, the percentage of nickel being less than 2.5 times the percentage of aluminum; said valve having the 115 characteristics of resistance to alteration in structure, size and shape with great temperature changes, retention of hardness and resistance to scaling at elevated temperatures, resistance to upsetting and to deformation under impact, and avoidance of seizure and galling of the valve stem in its guides.

120 3. A steel alloy comprising carbon about .2 to 1.25%, nickel about .5 to less than 4%, chromium about 6 to less than 15%, and aluminum 125 about .5 to 5%, the remainder being substantially iron.

130 4. A steel alloy comprising carbon about .2 to 1.25%, nickel about .5 to less than 5%, chromium about 6 to less than 15%, and aluminum 135 about .5 to 7%, the remainder being substantially iron.

140 5. A steel alloy comprising carbon about .2 to 1.25%, nickel about .75 to less than 4%, chromium about 6 to less than 10% and aluminum 145 about .5 to 5%, the remainder being substantially iron.

150

about 1 to 7%, the remainder being substantially iron.

6. A steel alloy comprising carbon about .2 to 1.25%, nickel about .5 to 7%, chromium about 6 to less than 15%, and aluminum about .5 to 7%, the remainder being substantially iron; the percentage of nickel not substantially exceeding the percentage of aluminum.

7. A steel alloy comprising carbon about .2 to 1.25%, nickel about .75 to less than 4%, chromium about 6 to less than 15%, and aluminum about 1 to 7%, the remainder being substantially iron; the percentage of aluminum being substantially in excess of the percentage of nickel.

10 8. A steel alloy comprising carbon about .2 to less than 1%, nickel about .5 to less than 5%, chromium about 6 to less than 15%, and aluminum over .3 and less than 7%, the remainder being substantially iron; the percentage of aluminum being not less than one-ninth of the percentage of chromium and nickel combined.

15 9. A steel alloy comprising carbon about .2 to 1.25%, nickel about .5 to less than 5%, chromium about 6 to less than 15% and aluminum over .3 and less than 7%, the remainder being substantially iron; the percentage of aluminum being not less than one-sixth the percentage of chromium and nickel combined.

20 10. A steel alloy comprising carbon about .2 to less than 1%, nickel about .75 to less than 4%, chromium about 6 to less than 15%, aluminum over .3 and less than 7%, the remainder being substantially iron; the percentage of aluminum being not less than one-ninth of the percentage of chromium and nickel combined.

25 11. A steel alloy comprising carbon about .2 to 1.25%, nickel about .75 to less than 4%, chromium about 6 to less than 15%, and aluminum over .3 and less than 7%, the remainder being substantially iron; the percentage of aluminum being not less than one-sixth the percentage of chromium and nickel combined.

30 12. A steel alloy containing carbon about .2 to .9%, nickel over .5 to less than 4%, chromium about 6 to less than 15%, and aluminum over 2 to less than 7%, the remainder being substantially iron.

35 13. A malleable steel resistant to hot oxidation containing effective amounts of chromium, nickel, and aluminum as essential alloying ingredients, the sum of the chromium and nickel contents ranging up to 18%, the nickel content being less than 5%, the chromium content being over 6% and less than 15%, and the aluminum content being over .3% and not over about 5%; the remainder being substantially iron.

14. A malleable steel resistant to hot oxidation containing effective amounts of chromium, nickel, and aluminum as essential alloying ingredients, the sum of the chromium and nickel contents ranging from 10 to 12.5%, the nickel content being less than 5% and the aluminum content ranging from 1.5 to 2%; the remainder being substantially iron.

15. A malleable steel resistant to hot oxidation containing effective amounts of chromium, nickel, and aluminum as essential alloying ingredients, the sum of the chromium and nickel contents ranging up to 18%, the chromium content being over 2%, the nickel content being less than 5%, and the aluminum content being between .3 and 3%; the remainder being substantially iron.

16. A malleable steel resistant to hot oxidation containing effective amounts of chromium, nickel, and aluminum as essential alloying ingredients, the sum of the chromium and nickel contents being less than 20%, the nickel content being less than 5%, the chromium content being over 2%, and the aluminum content being over .3% and not over about 5%; the remainder being substantially iron.

17. A hard steel alloy containing carbon .2 to 1.25%, nickel .5 to less than 5%, chromium 6 to less than 15%, and aluminum over .3 to less than 7%, the remainder being substantially iron, the percentage of nickel being less than 2.5 times the percentage of aluminum; said alloy having a critical temperature not less than about 1400° F. and having the characteristics of resistance to alterations in structure, size and shape with great temperature changes, retention of hardness at elevated temperatures, freedom from scaling, resistance to deformation, and which is readily malleable and machinable.

18. A hardened valve adapted for use in internal combustion engines and composed of a readily malleable and machinable steel alloy having a critical temperature not less than 1400° F. and containing nickel .5 to less than 5%, chromium 6 to less than 15%, and aluminum over .3 to less than 7%, the remainder being substantially iron, the percentage of nickel being less than 2.5 times the percentage of aluminum; said valve having the characteristics of resistance to alteration in structure, size and shape with great temperature changes, retention of hardness and resistance to scaling at elevated temperatures, resistance to upsetting and to deformation under impact, and avoidance of seizure and galling of the valve stem in its guides.

JOHN L. COX.

60

135

65

140

70

145

75

150